

## UNITED STATES PATENT OFFICE

1,942,173

## METHOD OF TREATING STEEL

Clarence I. Justheim, Salt Lake City, Utah

No Drawing. Application May 31, 1932  
Serial No. 614,630

3 Claims. (Cl. 75—27)

My invention relates to the treating of steel and has for its object to provide a new and efficient method of treating steel to produce a better quality steel than has heretofore been accomplished, producing a steel of greater tensile strength considering the low point of carbon content.

A further object is to provide a method of producing steel using a flux of carbonaceous deposit carrying a high content of silica.

A still further object is to produce a steel having greater ductility and producing such steel at less cost than by the known methods.

A still further object is to produce a steel having a better structure than the present day standard methods of making steel as revealed by the microscope.

A still further object is to provide a method of treating steel when in the molten state, which consists of introducing a flux forming a complete covering for the molten steel in the furnace or crucible, thereby prohibiting the entrance of gases or atmosphere.

These objects I accomplish with the following methods:

The steel producing mixture is introduced into the furnace or crucible and treated in the usual manner. Silica sand is used in all cases for the first slag to eliminate the first impurities, sufficient heat being used to produce the necessary result. The oxidized slag is then removed and a new slag formed, which in my case would consist of a carbonaceous shale deposit carrying a high percentage of silica. Then a quantity of ferromanganese is added. The resulting slag is removed and the metal poured as desired.

In some cases the use of the deoxidizing agent, such as ferromanganese, may be eliminated and the flux used in varying quantities either one or more times during the time of the melt, depending upon the type of steel desired.

The deoxidizing agent used may be ferromanganese, spiegeleisen, ferrosilicon, or any other suitable agent used in the present-day methods of making steel, depending upon the type of steel desired.

Ferromanganese, spiegeleisen, and ferrosilicon, are all deoxidizing agents of the type which must be prepared or manufactured for use, as they are alloys made by treating the materials of which they are composed, in a suitable manner to make them combine into the finished alloy for use in the process of making steel. In my process the manufactured alloy is introduced into the melt as before stated, by adding the ferromanganese or other alloy to the melt after the carbonaceous shale has been added, but in some cases the melt is made with the usual silica sand, slag formed, deslagged, and then the ferromanganese or manufactured deoxidizing agent is introduced and

later the cleaning and finishing slag is formed by the addition of my carbonaceous shale. This latter may be added to the melt after it is in the ladle, if desired.

The following tests were run in an electric furnace to prove the above specification. Five heats were made, of which number 1 was a present-day method. The steel making mixture used analyzed carbon 0.20 to 0.25%; manganese 0.60 to 0.75%; silicon 0.30 to 0.40%; phosphorus and sulphur 0.05% maximum. Silica sand was used in all cases for the first slag. This oxidizing slag was then removed and a new slag formed under the following conditions:

Heat No. 1— Silica sand, sufficient for steady arc  
Heat No. 2— 0.25 lb. of flux  
Heat No. 3— 0.12 lb. of flux  
Heat No. 4— 0.60 lb. of flux  
Heat No. 5— 1.00 lb. of flux

Just prior to tapping the following additions of 80% ferromanganese were added (no other deoxidizers were used in these tests):

| lb. Fe-Mn. | 85   |
|------------|------|
| Heat No. 1 | 0.25 |
| Heat No. 2 | 0.00 |
| Heat No. 3 | 0.12 |
| Heat No. 4 | 0.00 |
| Heat No. 5 | 0.00 |

The metal was then poured into test bars. The bars had the machining qualities typical to those having similar analysis and heat treatment.

## Results

| Heat No. | Fe-Mn lbs. | Flux lbs. | C    | Mn.  | Si.  | Yield Psi. | Ultimate Psi. | Elongation 2 inches 0.505" diameter | Reduction of area | Brinell | 100 |
|----------|------------|-----------|------|------|------|------------|---------------|-------------------------------------|-------------------|---------|-----|
| 1        | 0.25       | 0.00      | 0.70 | 0.77 | 0.44 | 100000     | 130750        | 7.05                                | 7.3               | 241     |     |
| 2        | 0.00       | 0.25      | 0.47 | 0.10 | 0.84 | 46250      | 77125         | 7.05                                | 7.3               | 170     |     |
| 3        | 0.12       | 0.12      | 0.50 | 0.33 | 0.58 | 59500      | 89875         | 10.15                               | 8.9               | 179     |     |
| 4        | 0.00       | 0.60      | 0.55 | 0.10 | 0.86 | 55750      | 77000         | 3.10                                | 3.5               | 187     |     |
| 5        | 0.00       | 1.00      | 0.68 | 0.13 | 1.02 | 41250      | 73000         | 2.30                                | 1.9               | 207     | 105 |

These results were obtained when carbonaceous shale from a deposit in Mesa County, Colorado, was used in the tests.

The use of this method protects the metal by forming a very tough glassy slag over the surface of the metal, preventing oxidation by the atmosphere and also further quiets the metal by the reaction of the nascent silicon with the nascent oxygen contained in the metallic bath. The nascent oxygen comes from two sources, metallic oxides, and the atmosphere. If there is not sufficient nascent silicon or other deoxidizing agents as ferromanganese present to react

110

115

120

with the nascent oxygen, it will remain in the steel in the form of metallic oxides or blow holes with the entrapped oxygen therein, either event weakening the steel.

5 The nascent silicon is the free atom or active atom liberated from the flux in the heat, and it is the state of the silicon in the flux which is responsible for the resulting metal.

An analysis of one portion of the flux showed 10 the following, being an average of several analyses:

|                | Percent  |
|----------------|----------|
| Silica         | 58.8     |
| Alumina        | 15.0     |
| 15 Iron oxide  | 3.1      |
| Sulphur        | .2       |
| Magnesia       | .8       |
| Lime           | .9       |
| Alkalies       | 1.8      |
| 20 Moisture    | 3.0      |
| Ignition loss  | 16.4     |
| Radio activity | None     |
| Vanadium       | No trace |
| Uranium        | No trace |

25

30

35

40

45

50

55

60

65

70

75

Having thus described my invention I desire to secure by Letters Patent and claim:

1. A method of making steel in which carbonaceous shale is used as a natural deoxidizing agent in combination with a manufactured de- 80 oxidizing agent to form the slag and produce steel having greater tensile strength, greater Brinell hardness, and greater elongation at less cost.

2. In a process for making steel the steps of melting a steel producing charge in the presence of a siliceous slag, removing the slag, and placing upon the metal a carbonaceous shale ranging from 40 to 70 percent silica and heating the same to form a second clearing slag and to precipitate nascent silicon into the steel and then deoxidizing the melt. 85

3. In a process for making steel the steps of melting a steel producing charge in the presence of a siliceous slag, removing the slag, and placing upon the metal a carbonaceous shale, ranging from 40 to 70 percent silica, and heating the same to liberate nascent silicon and form a clearing slag. 90

CLARENCE I. JUSTHEIM. 100

105

110

115

120

125

130

135

140

145

150